

1

2,894,909

**SYNTHETIC LUBRICANT**

Charles E. Saunders, Silver Spring, Md., assignor to United States of America as represented by the Secretary of the Navy

No Drawing. Application August 9, 1956  
Serial No. 603,196

3 Claims. (Cl. 252—34.7)

(Granted under Title 35, U.S. Code (1952), sec. 266)

The invention described herein may be manufactured and used by or for the Government of the United States of America for governmental purposes without the payment of any royalties thereon or therefor.

The present invention relates to synthetic lubricants and additives therefor. More particularly the invention relates to water soluble polymerized alkylene oxide oils and to additives which improve the lubricity and antioxidant characteristics of these oils so as to make them useful under extreme ambient conditions while retaining their water soluble characteristics.

This application is a continuation-in-part of Serial No. 241,379, filed August 10, 1951, now abandoned.

Improved high powered turbine type internal combustion engines have recently been developed for use in high speed underwater ordnance equipment such as submarines and torpedoes. An example of this type of engine is the hydrogen peroxide propelled engine used in submarines. This engine is combined with the conventional diesel engine with the peroxide reserved for special bursts of speed in attacking and escaping. Free oxygen combines with fuel such as diesel oil to produce the steam and carbon dioxide to drive the turbine under ordinary conditions. When high speed is desired the hydrogen peroxide is utilized as the fuel. The hydrogen peroxide breaks down to provide the heat used as the source of energy. The principal advantage of the use of hydrogen peroxide is that no exhaust bubbles reach the surface thus adding a safety factor to the submarine's operation. The hydrogen peroxide engine, however, develops temperatures in the nature of 1200 degrees F. so that it is highly desirable to utilize sea water as a coolant. This sea water coolant tends to wash away the lubricants employed in the engine and such lubricants are discharged with the sea water. Ordinary lubricants being insoluble in sea water tend to form a wake in the form of an oil slick which rises to the surface. The presence of this slick may be detected by surface craft and the advantage the submarine has obtained through the use of the hydrogen peroxide engine is largely overcome. In addition ordinary lubricants tend to wash off the engine parts in the presence of sea water. They also are extremely corrosive or tend to break down at high temperatures in the presence of the steam and free oxygen employed in the engines.

Many mineral oils, compounded heavy duty oils and synthetic oils have been extensively tested in an effort to eliminate this slick type of wake while retaining the necessary high lubricity and anticorrosive characteristics required for use in the engines of the hydrogen peroxide type. The results of these tests showed that to perform as required, a lubricant must be either water soluble or have a specific gravity considerably greater than that of sea water. These characteristics must be retained even after the lubricant has been subjected to the rigors of the high temperatures developed in the combustion chamber of hydrogen peroxide engines or the like.

2

Of the many oils tested only the water soluble oils formed by the polymerization of alkylene oxides have been found to have characteristics which approach those found to be necessary for use under the above described conditions. These water soluble polymerized alkylene oxide oils have lubricity characteristics which compare favorably with conventional petroleum oils. They are superior to most petroleum oils with regard to viscosity index, pour point and sludge formation. However, these alkylene oxide oils have been found to give inadequate lubrication under the conditions of operation described for the hydrogen peroxide engine and have been found to be unduly corrosive when compared to hydrocarbon oils.

Attempts to improve the lubricity and anticorrosive characteristics of the polymerized alkylene oxide oils while retaining their water soluble, slick free qualities have not heretofore been successful. All previously known additives either do not improve the lubricity and anticorrosive characteristics of the oils or result in the lubricant forming the highly undesirable slick. It is therefore, an object of the present invention to provide a new and improved additive for use with alkylene oxide oils.

Another object is to provide a new and improved alkylene oxide lubricating compound having improved lubricity and anticorrosive characteristics.

A further object is to provide a new and improved lubricating composition which is soluble in water and will not form a slick when used under water.

A still further object is to provide an additive for improving the lubricity characteristics of alkylene oxide oils while decreasing their corrosiveness.

Other objects and the attendant advantages of the invention will be apparent to those skilled in the art as the invention is disclosed in the following detailed description.

The objects of the present invention are achieved by the addition to the alkylene oxide oil of a small proportion of ammonium linoleate. The addition of as small a quantity of ammonium linoleate as 1-2 percent by weight permits satisfactory lubrication of an internal combustion engine even when 50 percent of sea water is present in the crankcase of the engine. The addition of this small proportion of ammonium linoleate also permits the use of the mixture as a steam cylinder lubricant.

The ammonium linoleate which is used in the invention has the formula  $\text{NH}_4\text{C}_{17}\text{H}_{31}\text{CO}_2$  and may be prepared by any of several well known methods such as the ammonialysis of linoleic acid. Ammonium linoleate is commercially available and any reasonably pure product may be utilized in the composition of this invention.

The alkylene oxide oils used in the lubricating composition of the invention are the oils composed of the water soluble polymerized ethylene glycols and derivatives thereof. These oils are commercially available under the trade name Ucon Lubricants from the Carbide and Carbon Chemicals Company. Only the water soluble oils are useful in the composition of this invention however. Ucon HB series lubricants are water soluble oils made by copolymerizing a mixture of ethylene oxide ( $\text{C}_2\text{H}_4\text{O}$ ) and propylene oxide ( $\text{C}_3\text{H}_6\text{O}$ ). These oils, being water soluble, form no slick on the surface of

water. They do not carbonize in the engine as badly as petroleum oils but are depolymerized forming water soluble glycols, acids and aldehydes leaving an exceptionally clean engine. These oils may be polymerized to any desired viscosity. Of the Ucon HB series lubricants Ucon 50 HB 660 is the preferred lubricant. This oil is made by copolymerizing a 50-50 mixture of ethylene oxide

and propylene oxide. As commercially available Ucon 50 HB-660 has the following properties:

Viscosity, SSU at:

|                                          |         |
|------------------------------------------|---------|
| 210 degrees F-----                       | 123     |
| 100 degrees F-----                       | 660     |
| 20 degrees F-----                        | 9,430   |
| 0 degrees F-----                         | 30,800  |
| -20 degrees F-----                       | 122,400 |
| -40 degrees F-----                       | 733,000 |
| V.I. (ASTMD-567-41)-----                 | 144     |
| Pour point (ASTM D-97-39) degrees F----- | -55     |

Sp. gr. at:

|                                                |       |
|------------------------------------------------|-------|
| 210 degrees F. g./cc-----                      | 0.985 |
| 100 degrees F. g./cc-----                      | 1.030 |
| 60 degrees F. g./cc-----                       | 1.047 |
| Min. flash point (ASTM D 92033) degrees F----- | 450   |
| Min. fire point (ASTM D 97033) do-----         | 500   |

Mere mechanical mixing of the ammonium linoleate with the Ucon lubricant oil will allow some separation of the constituents after prolonged standing at room temperature.

A permanent colloidal suspension of the ammonium linoleate may best be prepared by first mixing the ammonium linoleate with the oil dissolving it in carbon tetrachloride and then adding this solution to the warmed oil with stirring. The carbon tetrachloride may then be removed by warming the mixture.

The following example is given by way of illustration and is not to be construed as limiting the invention in any manner.

#### EXAMPLE I

A mixture of Ucon 50 HB 660 and ammonium linoleate was prepared by dissolving the ammonium linoleate paste in carbon tetrachloride at 90 degrees F. This solution was added to the Ucon 50 HB 660 at 135 degrees F and stirred for fifteen minutes. The carbon tetrachloride was removed by heating the mixture to 200 degrees F. under a vacuum.

The test for the formation of an oil slick was performed on a one cylinder, four stroke cycle, Lauson gasoline engine so modified as to give a condition of excessive oil consumption. For this purpose the oil control ring was removed from the piston leaving only the two compression rings. A mixture of hydrogen, oxygen and steam was used as the fuel. The exhaust from the engine was piped to the lowest point of a tank holding 15 gallons of synthetic sea water about four feet deep. A baffle plate with small holes was placed above the exhaust line to distribute the gases throughout the tank area.

Straight mineral oils and compounded heavy duty oils formed objectionable oil slicks on the water surface with the above test. Various synthetic oils were also tested including glycerin, tricresyl phosphate, Hydrolubes, Ucon LB series, Arochlor 1278, Gulf Oeca and Dow Corning Fluids #200, #710 and #500. All the oils tested gave unsatisfactory results except the Ucon HB series. When Ucon 50 HB 660 plus the ammonium linoleate was tested the entire products of the exhaust were soluble in the water and left no slick on the surface.

The mixture of Ucon 50 HB 660 and ammonium linoleate was tested for comparison with other lubricants on a wear test machine. The testing machine used to test the oils was a constant speed (1800 r.p.m.) motor with a hardened steel wheel attached to the shaft. This wheel was hardened to Rockwell 60c. The motor was attached to a base plate which held a lever arrangement that permitted loading of the test piece. The test pieces were cold rolled steel  $\frac{1}{2}$ " x 2" x  $\frac{3}{16}$ ". The loading was accomplished by using the lever arrangement to force the test piece against the wheel. A 5:1 lever ratio gave a 20 pound loading at the point of contact. The

tested lubricant was fed from a drip oiler so it just contacted the edge of the wheel as it was fed.

The test was started by allowing the oil to completely cover the sample and to flow at an arbitrary drip rate (about 90 drops per minute) which was maintained for the duration of the run. The sample was allowed to come into contact with the wheel and the test was allowed to run for 5 minutes. The test was secured by removing the sample from contact with the wheel. The resultant length of the mark on the test sample served as a comparative measurement of the quality of the lubricant tested.

A petroleum base oil SAE 30 blended with 20 percent of brown rape seed oil was used as a standard for comparison since this mixture of oils was found to permit engine operation in the presence of sea water, oxygen and steam as described above even though the lubricating qualities of the oil appeared to be marginal and it caused a bad oil slick.

For the purpose of the tests each of the oil samples tested was diluted with an equivalent amount of synthetic sea water so as to produce a lubricant containing 50 percent sea water.

Table I shows the averages obtained from a series of wear tests on the Ucon 50 HB 660 without additive, on the Ucon 50 HB 660 plus 2% ammonium linoleate and on the standard petroleum base oil.

Table I

|                                                | Wear in in. 20# wt. |
|------------------------------------------------|---------------------|
| Pet base oil SAE 30-----                       | .1200               |
| UCON 50 HB 660-----                            | .2299               |
| UCON 50 HB 660 plus 2% ammonium linoleate----- | .1050               |

The results of the wear test showed that the Ucon 50 HB 660-ammonium linoleate mixture had better lubricating qualities than the standard petroleum base oil and showed a reduction of over 50 percent of wear over Ucon 50 HB 660 without additive.

The Ucon 50 HB 660-ammonium linoleate mixture was subjected to a storage test. The ammonium linoleate remained in suspension at -50 degrees F. and after 6 months at 150 degrees F.

The anticorrosive characteristics were found to be satisfactory. The neutralization numbers i.e. the number of mg. of potassium hydroxide required to neutralize one gram of oil are as follows

|    | Originally | 2 wks. | 4 wks. | 6 wks. |
|----|------------|--------|--------|--------|
| 50 | 3.36       | 3.30   | 2.91   | 3.14   |

From the foregoing it may be seen that there has been provided a synthetic lubricant composition which has lubricative characteristics comparable to or better than the best petroleum oils when mixed with up to 50 percent sea water and which is water soluble even after being subjected to the high temperatures of the combustion chamber of an internal combustion engine and which accordingly forms no undesirable slick on the water. This improved lubricating composition composed of copolymerized ethylene oxide and propylene oxide with up to 2% ammonium linoleate has been employed successfully with no corrosive results in submarine and torpedo engines of the hydrogen peroxide type.

Obviously many modifications and variations of the present invention are possible in the light of the above teachings. It is therefore to be understood that within the scope of the appended claims the invention may be practiced otherwise than as specifically described.

What is claimed as new and desired to be secured by Letters Patent of the United States is:

1. A water soluble lubricating composition comprising

a water soluble polymerized alkylene oxide oil consisting of ethylene oxide and propylene oxide, and substantially 2 percent by weight of ammonium linoleate.

2. A water soluble lubricating composition comprising an alkylene oxide oil containing substantially 50 percent by weight of polymerized ethylene oxide and 50 percent by weight of polymerized propylene oxide, and an additive consisting of substantially 2 percent by weight of ammonium linoleate.

3. A water soluble lubricating composition comprising a water soluble alkylene oxide oil consisting substantially in a 1:1 ratio of copolymerized ethylene oxide and propylene oxide, and having substantially 2 percent by weight of ammonium linoleate mixed therein.

10

## References Cited in the file of this patent

## UNITED STATES PATENTS

|           |          |               |
|-----------|----------|---------------|
| 1,414,227 | Sorenson | Apr. 25, 1922 |
| 1,881,173 | Dahlberg | Oct. 4, 1932  |
| 2,162,454 | Guthman  | June 13, 1939 |
| 2,587,546 | Matuszak | Feb. 26, 1952 |
| 2,624,708 | Langer   | Jan. 6, 1953  |

## OTHER REFERENCES

"Ucon," Carbide and Carbon Chem. Corp., N.Y. (1948), Table No. 3, between pages 10 and 11.  
 "Ind. and Chem. Eng.," vol. 40, No. 12, page 2346.